

## UNITED STATES PATENT OFFICE

2,474,617

## MANUFACTURE OF ARTIFICIAL FIBERS

Edward Terry Cline, Wilmington, Del., assignor  
to E. I. du Pont de Nemours & Company, Wil-  
mington, Del., a corporation of Delaware

No Drawing. Application January 3, 1947,  
Serial No. 720,099

5 Claims. (Cl. 18—54)

1

This invention relates to the production of artificial fibers, and more particularly to an improved process for the manufacture of fibers of hydroxyl-containing polymers obtained by wet-spinning.

Fibers previously have been prepared from highly hydroxylated polymers such as polyvinyl alcohol. These fibers have many advantages. They can be oriented to give filaments and yarns of high tensile strength. They possess advantageous insolubility in common organic solvents such as are used in the dry-cleaning industry. Furthermore, they are high softening and are useful for applications such as in tire cords and ironable fabrics where resistance to heat is necessary. Filaments have been prepared by the dry-spinning of aqueous solutions such as by the rapid evaporation of the aqueous solvent when a fine stream of the aqueous polymer solution is injected into a heated chamber. However, for such advantages as uniformity, ease of spinning yarns of high denier, and inexpensive mechanical equipment requirements, wet spinning of aqueous solutions is preferable. This involves injecting an aqueous solution of the polymer into a coagulating bath. This method, however, has been accompanied by a serious disadvantage in that when the fibers are prepared by spinning an aqueous solution of the polymer into a saturated aqueous solution of an inorganic salt such as  $\text{NaH}_2\text{PO}_4$  to coagulate the fiber, considerable difficulty is encountered in removing the salt from the fiber. Water is the best solvent for the salt. However, in view of the water sensitivity of the hydroxyl-containing polymer, an aqueous wash to remove the salt tends to dissolve the fibers and they become tacky when the salt concentration in the water becomes low. After the fibers have been allowed to dry, they are found to be stuck together and therefore unusable.

A method for removing salts has been shown in U. S. Patent 2,388,325 in which water-organic solvent mixtures such as a 1:1 mixture of water and acetone, are used to remove salts from polyvinyl alcohol structures freshly precipitated from aqueous inorganic salt solutions without injurious effect. Such a method is expensive and the aqueous organic solution is less effective than water to extract water-soluble salts in view of the low solubility of the coagulating bath salts in organic solvents.

An object of this invention is an improved process for the removal of inorganic salts from coagulated hydroxyl-containing polymer structures which are obtained by injection of the polymer in a salt-containing coagulating bath. Other objects will appear hereinafter.

2

The above objects are accomplished by a procedure more particularly described below which comprises drawing under tension the wet spun filaments of a synthetic linear hydroxylated polymer having at least one alcoholic hydroxyl group per 2.5 carbons and not more than one hydroxyl per two carbons of the polymeric chain, holding the filaments at a length of at least twice their original length, washing with water while the filaments are held at at least twice their original length to remove the coagulating bath salts from the filaments, and drying while so maintained.

The terms "original" or "initial length" as employed herein mean the length after coagulation of the filaments. When no rollers or other tensioning devices are employed in the coagulating bath, this length is that of the yarn as it leaves the bath. When yarn driven rollers are used in the coagulating bath, this length is that of the yarn at the time it encounters the first coagulating bath roller.

The following examples in which the parts given are by weight further illustrate this invention.

## EXAMPLE I

An aqueous solution containing 15% of a hydrolyzed ethylene/vinyl acetate interpolymer containing about 5% ethylene in the hydrolyzate, was extruded by means of a gear pump through a multi-hole viscose rayon type spinneret into a coagulating bath containing 45% monosodium dihydrogen phosphate and 0.05% "Retarder" LA (20% octadecyltrimethylammonium bromide). From the coagulating bath the yarn was led to a positively driven Godet, a six inch diameter glass wheel fitted with an idler roller so that several yarn wraps could be taken around the wheel to avoid slippage. The yarn was then led through air to a positively driven wind up bobbin. By adjusting the speeds of the various drives, the yarn could be stretched in controllable amounts either in the coagulating bath or in air between the Godet and wind up or both. It was found preferable to pass the yarn in the coagulating bath around one or more rollers mounted on vertical posts in the bath before the yarn was led to the Godet or directly to the wind up.

During the course of the spinning, some of the yarns were subjected to various degrees of stretch in the coagulating bath as calculated from the speed of the yarn as it left the bath and the peripheral speed of the first roller in the bath. Others were stretched only slightly in the bath but were stretched various degrees in air between the Godet and wind up. Where yarn driven rollers were used in the coagulating

bath, the total stretch applied to the yarn was calculated from the peripheral speed of the first bath roller and the speed of the wind up bobbin. Where no rollers were used in the coagulating bath, the total stretch was calculated from the peripheral speed of the Godet wheel and the speed of the wind up bobbin. These calculations neglect any stretch applied to the yarn between the spinneret and first roller, or where no rollers were used, any stretch occurring in the coagulating bath. The yarn may be stretched to a small extent in these regions as a result of friction between the yarn and the bath or any stationary object which the yarn may touch such as a convergence guide. In practice, however, this stretch is relatively insignificant in view of the fact that the orientation of the yarn at this stage is low as evident from measurement of its orientation number as defined in the following paragraph. A coagulating bath temperature of 60° C. was used during part of the spinning. For each condition used, the tension on the yarn just before the wind up bobbin was measured in grams and later calculated in terms of g. p. d. (grams per denier). After each bobbin of yarn had been collected, it was washed in running tap water until the coagulating bath salts were substantially removed. It was then allowed to dry in air and the condition of the yarn, i. e., whether stuck or free, was observed. Free yarns were twisted on a conventional ring twister. Short lengths of the stuck yarns were unwound laboriously by hand during which many of the individual filaments were broken. The orientation numbers of the yarns were then determined by means of X-rays.

Orientation is determined by passing a collimated beam of copper filtered X-radiation through a bundle approximately 1 mm. thick of parallel fibers onto a photographic plate during one hour with a distance of 5 cm. between the fiber specimen and the plate. The Phillips Metalix tube used is supplied with a 19 milliampere current at 35 kilovolts. The collimation is effected by two 25-mil diameter pinholes separated by a distance of 8 cm. The filter thickness is 0.6 mil. The X-ray negative is developed and analyzed photometrically. From the density of silver deposit at any given point in the negative, the intensity of X-rays impinging on that point during exposure can be calculated. The extent of orientation of the specimen is expressed in terms of the ratios of the calculated X-ray intensities at the equator of the picture to that at 90 degrees from the equator for the inner and outer rings. The ratios are called orientation numbers. Thus an orientation number of one denotes that the specimen shows no orientation whereas ratios progressively greater than one denote progressively higher degrees of orientation. The orientation numbers are expressed as  $O_1$  for the inner ring and  $O_2$  for the outer ring of the X-ray diffraction pattern. Of these the  $O_2$  orientation number is more accurate and reproducible. These values are given in the examples.

It was found that if the yarns were arranged in order of increasing amount of total stretch, they were also in order of increasing orientation number and increasing wind up tension as expressed in grams per denier. The yarns collected below a total stretch of about 100% of their original length were stuck whereas those collected above this total stretch were sufficiently

resistant to water so that they could be washed with water and dried without becoming stuck together. Likewise the yarns collected below a given wind up tension or below a given orientation number were stuck whereas those collected above this critical wind up tension or orientation number were not stuck. Washing and drying of these yarns was carried out at constant yarn length on the wind-up bobbins. If the yarns are removed from the bobbins and allowed to relax completely during washing and drying, as in a skein, they will shrink freely, lose orientation and become stuck. It was found that the place at which the stretch is applied during spinning, i. e., in the coagulating bath or in air outside the coagulating bath, is immaterial in regard to washability. Typical results obtained in this spinning are shown in the following tables.

Table I

| Amount Yarn<br>Stretched in— |         |         | Total<br>Stretch | Washed and Dried<br>Yarn Condition |
|------------------------------|---------|---------|------------------|------------------------------------|
| Coag.<br>Bath                | Air     | Percent |                  |                                    |
| Percent                      | Percent | Percent |                  |                                    |
| 29                           | 0       | 29      |                  | Badly stuck.                       |
| 57                           | 0       | 57      |                  | Do.                                |
| 6                            | 61      | 70      |                  | Do.                                |
| 72                           | 0       | 72      |                  | Partly stuck.                      |
| 78                           | 0       | 78      |                  | Do.                                |
| 90                           | 0       | 90      |                  | Do.                                |
| 104                          | 0       | 104     |                  | Free.                              |
| 6                            | 101     | 112     |                  | Do.                                |
| 115                          | 0       | 115     |                  | Do.                                |
| 124                          | 0       | 124     |                  | Do.                                |
| 6                            | 239     | 258     |                  | Do.                                |
| 422                          | 0       | 422     |                  | Do.                                |

Table II

| Amount Yarn<br>Stretched in— |     | Wind up<br>Tension,<br>g. p. d. | Washed and<br>Dried Yarn,<br>Condition | Orien-<br>ta-<br>tion<br>No. $O_2$ |
|------------------------------|-----|---------------------------------|----------------------------------------|------------------------------------|
| Coag.<br>Bath                | Air | Percent                         | Percent                                |                                    |
| 6                            | 28  | 0.026                           | Stuck                                  |                                    |
| 6                            | 61  | 0.040                           | Do                                     | 2.4                                |
| 25                           | 0   | 0.045                           | Do                                     | 2.5                                |
| 115                          | 0   | 0.051                           | Free                                   | 2.4                                |
| 78                           | 0   | 0.071                           | Do                                     | 2.8                                |
| 222                          | 0   | 0.085                           | Do                                     | 3.0                                |
| 104                          | 0   | 0.114                           | Do                                     | 3.5                                |
| 6                            | 138 | 0.123                           | Do                                     | 4.9                                |

The critical wind up tension and  $O_2$  orientation number (ratio of X-ray intensity at the equator to that at the pole for the outer interference ring) for this yarn may be seen to lie between 0.05 and 0.07 g. p. d. and between 2.4 and 2.8 respectively.

## EXAMPLE II

An aqueous solution containing 13.5% of medium viscosity polyvinyl alcohol having a saponification number of 3 and a viscosity of 20.9 centipoises (4% aqueous solution) was spun in a manner similar to that described in Example I. For most of the yarns collected, practically all of the stretching was done in air between the Godet and wind up. In order to avoid sticking during washing and drying it was necessary to apply a total stretch of about 190% to these yarns. The maximum possible stretch was approximately 400%. As was the case in Example I, the yarns when arranged in order of increasing stretch and wind up tension, also were in order of increasing orientation numbers. Thus,

## 5

for the polyvinyl alcohol yarns, it was necessary that the total stretch be higher (correspondingly, a higher wind up tension with higher orientation number) to permit washing and drying without sticking than in the case of the hydrolyzed ethylene/vinyl acetate interpolymer yarns described in Example I. It is therefore evident that polyvinyl alcohol is more water sensitive than hydrolyzed ethylene/vinyl acetate interpolymers.

Typical results obtained in this spinning are 10 shown in the following tables.

Table III

| Amount Yarn Stretch in— |          | Total Stretch | Washed and Dried Yarn, Condition |
|-------------------------|----------|---------------|----------------------------------|
| Coag. Bath              | Air      |               |                                  |
| Per cent                | Per cent | Per cent      |                                  |
| 15                      | 59       | 83            | Stuck.                           |
| 16                      | 87       | 116           | Do.                              |
| 16                      | 111      | 144           | Do.                              |
| 16                      | 139      | 176           | Do.                              |
| 6                       | 180      | 196           | Free.                            |
| 16                      | 186      | 208           | Do.                              |
| 16                      | 194      | 240           | Do.                              |
| 5                       | 267      | 286           | Do.                              |
| 11                      | 267      | 308           | Do.                              |

Table IV

| Amount Yarn Stretched in— |          | Wind Up Tension, g. p. d. | Washed and Dried Yarn, Condition | Orientation No. O <sub>2</sub> |
|---------------------------|----------|---------------------------|----------------------------------|--------------------------------|
| Coag. Bath                | Air      |                           |                                  |                                |
| Per cent                  | Per cent |                           |                                  |                                |
| 16                        | 111      | 0.12                      | Stuck.....                       | 3.7                            |
| 16                        | 139      | .15                       | do.....                          | 4.6                            |
| 16                        | 166      | .21                       | Free.....                        | 5.5                            |
| 16                        | 194      | .30                       | do.....                          | 6.3                            |
| 5                         | 267      | .87                       | do.....                          | 8.1                            |

The critical wind up tension and O<sub>2</sub> orientation number for this yarn may be seen to lie between 0.15 and 0.21 g. p. d. and between 4.6 and 5.5 respectively.

The ethylene present in the hydrolyzed ethylene/vinyl acetate interpolymer appears to be responsible for its greater water resistance over polyvinyl alcohol. To avoid sticking in a bobbin process, the total stretch for polyvinyl alcohol is at least 190% and for a hydrolyzed vinyl acetate interpolymer containing 5% ethylene is 100%. Each per cent of ethylene introduced lowers the amount of total stretch by 18 from the 190%. Correspondingly, if the upper limits of the critical ranges of wind up tension and O<sub>2</sub> orientation number given in Examples I and II are taken as the critical points, then each percent of ethylene introduced lowers the wind up tension about 0.03 g. p. d. and the O<sub>2</sub> orientation number by about 0.5 without encountering sticking in the washed and dried yarn. This is illustrated in the following table.

Table V

| Polymer                                                       | Critical Wind up Tension (g. p. d.) | Critical Orientation No. (O <sub>2</sub> ) | Critical Stretch |
|---------------------------------------------------------------|-------------------------------------|--------------------------------------------|------------------|
|                                                               |                                     | Per cent                                   |                  |
| Polyvinyl alcohol                                             | 0.21                                | 5.5                                        | 190              |
| Hydrolyzed ethylene vinyl acetate containing 5% ethylene..... | .07                                 | 2.8                                        | 100              |
| Difference.....                                               | .14                                 | 2.7                                        | 90               |
| Difference $\times \frac{1}{18}$ .....                        | .03                                 | 0.5                                        | 18               |

## 6

## EXAMPLE III

An aqueous solution containing 7% ethanol and 15.4% of hydrolyzed ethylene/vinyl acetate interpolymer containing 5% ethylene was spun in a manner similar to that described in Example I. The spinning solution was delivered through a 60 hole spinneret at a rate of 3 cc. a minute. In the coagulating bath, which was maintained at room temperature, the yarn was passed around 2 rollers such that the length of yarn travel in the bath was about sixty inches. The yarn was then led to a Godet wheel operating at a peripheral speed of 380 inches per minute. It was then led thru air to the wind up bobbin, operating at a peripheral speed of 1380 inches per minute, such that it was stretched in air 263% (or a draw ratio of 3.63/1). The wind up tension was 0.58 g. p. d. Following washing and drying of the yarn, the filaments were observed not to be stuck.

## EXAMPLE IV

An aqueous solution containing 7% ethanol and 12.5% of high viscosity, fully hydrolyzed PVA (polyvinyl alcohol) having a viscosity of 51 centipoises (4% solution in water) was spun in a manner similar to that described in Example III. The spinning solution was delivered to the spinneret at a rate of 4.5 cc. per minute. Following passage around two rollers in the coagulating bath, the yarn was led to a Godet wheel operating at a peripheral speed of 285 inches per minute. From the Godet the yarn was led to the wind up bobbin operating at a peripheral speed of 1040 inches per minute such that it was stretched in air 265%. The wind up tension was 0.48 g. p. d. Following washing and drying the yarn could be unwound readily and the filaments were not stuck together.

## EXAMPLE V

An aqueous solution containing 7% ethanol, 0.7% sodium hydroxide, 1.1% carbon disulfide and 5% of a hydrolyzed ethylene/vinyl acetate interpolymer containing about 11% ethylene was spun in a manner similar to that described in Example I except that a viscose rayon type coagulating bath containing sodium sulfate, zinc sulfate and 4% sulfuric acid was employed. During spinning samples of yarn were stretched in air 114% and other samples 250%. In both cases the yarn following washing with water and drying was found to be free from sticking.

## EXAMPLE VI

An aqueous solution containing 7.3% ethanol and 15.4% of a hydrolyzed ethylene/vinyl acetate interpolymer containing about 5% ethylene was spun in a manner similar to that described in Example I except that a boiling aqueous bath containing 20% urea was used between the Godet and the wind up such that the yarn passed thru this solution while it was being stretched between the Godet and wind up. Most of the yarn was collected at a total stretch of 520%. The maximum possible stretch was 600%. The water washed and dried yarn was not stuck.

## EXAMPLE VII

An aqueous solution containing 14% of polyvinyl alcohol was spun in a manner similar to that described in Example I except that a simulated bucket type wind up was employed. From the Godet wheel the yarn was led to a positively 75 driven draw roll and thence to a wind up bobbin.

The wind up bobbin was operated at a lower peripheral speed than the draw roll such that the yarn was relaxed a controlled amount between the draw roll and the wind up. The total stretch was calculated from the peripheral speed of the final wind up bobbin and the yarn speed at the first coagulating bath roller in spite of the fact that the yarn was actually stretched more than this prior to its relaxation between the draw roll and the wind up bobbin. Following winding the yarn was washed with water, allowed to dry in air and, twisted. The results on yarns spun under several different conditions of stretch are shown in the following table.

| Spinning Speeds, Inches/Minute |       |           |         | Tensions, g. p. d. <sup>1</sup> |            | Total Stretch | Condition of Final Yarn |
|--------------------------------|-------|-----------|---------|---------------------------------|------------|---------------|-------------------------|
| No. 1 Coag. Bath Roller        | Godet | Draw Roll | Wind up | At Draw Roll                    | At Wind Up |               |                         |
| 332                            | 340   | 1,140     | 1,030   | .49                             | .04        | 210           | Partly stuck.           |
| 350                            | 377   | 1,384     | 1,108   | .76                             | .02        | 216           | Do.                     |
| 350                            | 377   | 1,380     | 1,163   | .58                             | .04        | 229           | Free.                   |
| 360                            | 377   | 1,384     | 1,210   | .84                             | .08        | 246           | Do.                     |
| 350                            | 377   | 1,500     | 1,280   | -----                           | .06        | 266           | Do.                     |

<sup>1</sup> g. p. d. = grams per denier.

It is apparent that yarns spun in this manner, i. e., by stretching them and then relaxing them controlled amounts before winding, must be given a somewhat higher total stretch than yarns spun by the bobbin process without relaxation as described in previous examples. Thus the total net stretch required to avoid sticking of the polyvinyl alcohol fibers described in this example is about 220% whereas only about 190% total stretch was required for the process described in Example II.

It is necessary however that the polyvinyl alcohol filaments be drawn at least 2.9 times their original length and maintained during the time they are in contact with water (e. g., during washing) at a length of at least 2.9 times their original undrawn length. If the filaments are drawn more than 2.9 times their original length, they must be maintained during the time they are in contact with water at their drawn length or at least 3.2 times their original length.

The macromolecular synthetic polymers that can be used in the process of this invention are those which have at least one alcoholic hydroxyl group per 2.5 carbon atoms but not more than one hydroxyl for two carbon atoms of the chain. By "macromolecular" is meant an organic compound having a degree of polymerization or a number of recurring units of at least 100 (Staudinger, Die Hochmolekularen Organischenen Verbindungen, 1932). Such hydroxyl-containing polymers include polyvinyl alcohol and hydrolyzed polyvinyl ester polymers and copolymers which have the ratio of hydroxyl to chain carbon previously mentioned. In addition to the hydrolyzed polyvinyl esters such as polyvinyl acetate, hydrolyzed copolymers of vinyl esters with ethylene, vinyl chloride, vinyl fluoride, vinylidene fluoride, vinylidene chloride, and other fiber-forming polymeric material can be employed. In such copolymers, the molar ratio of vinyl ester (hydrolyzed to vinyl alcohol) to the other polymerizable compounds is preferably between 6:1 and 50:1. Of the hydroxylated polymers those particularly preferred are polyvinyl alcohol and hydrolyzed ethylene-vinyl ester interpolymers, containing from 0.12% to 10.0% ethylene in the hydrolyzate. The preparation of the latter interpolymers has been de-

scribed in U. S. Patent 2,386,347. These polymers have been there characterized by the empirical formula:



where R is an acyl radical of an organic monocarboxylic acid, preferably acetyl and the ratio of y to z is at least 4 to 1 (i. e., 80% hydrolyzed) and preferably substantially completely hydrolyzed. For polyvinyl alcohol, x is zero while for the ethylene interpolymers, the ratio of y+z to x is usually within the range of 6:1 to 50:1 and is preferably 6:1 to 25:1 since the fibers from the latter polymers have better properties.

The above polymers are dissolved in hot aqueous solution to an extent of between 5 and 30% although usually between 5 and 20% is used. There may be also added small amounts of water-soluble aliphatic alcohols, amines, or mercaptans. For difficultly soluble polymers, mixtures of an alkali metal hydroxide and carbon disulfide are desirable. Such adjuvants are useful in preparing solutions of better homogeneity for extrusion through spinnerets into the coagulating bath. The coagulating bath is an aqueous solution of one or more inorganic alkali metal salts such as sodium sulfate, disodium hydrogen phosphate, zinc sulfate, potassium sulfate, ammonium chloride, etc. Particularly desirable in view of the better coagulating properties (effectiveness in removing water from the polymer solution) is an aqueous coagulating bath consisting of monosodium dihydrogen phosphate ( $NaH_2PO_4$ ) having a specific gravity of about 1.4 at 25° C. The salt bath should have a high concentration, e. g., it should be nearly saturated with salt or of sufficient concentration to remove water rapidly from the aqueous polymer solution. Cationic surface active agents such as cetyl trimethyl pyridinium bromide in amounts of from 0.005 to 0.05% based on the weight of the bath are also advantageous in that the filaments have improved properties and spinnerets are less likely to foul. Cationic surface active agents are described in British Patent 499,334. Usually the bath is saturated with respect to the surface active agent. The bath is usually maintained at temperatures of 5 to 80° C.

The drawing or stretching of the filaments with resulting molecular orientation along the fiber axis is conducted under a tension which draws them to a length of at least twice their initial length and which orients the filaments to an extent that when held at fixed length they are insufficiently softened by water to cause sticking of the dried filaments. Although in all instances the tension applied draws them to a length of at least twice their initial length, or is at least 0.05 gram per denier, the exact amount of orientation necessary will depend on the water sensitivity of the particular polymer, and the minimum tension will, therefore, be higher for the more water

sensitive polymers. This figure can be obtained readily by trial or by the rule given below for approximating the minimum tension that should be applied to orient the fiber so that it can be washed with water and dried.

For a polymer represented by the empirical formula  $(C_2H_3OH)_a (C_2H_4)_b$ , the first member being the polyvinyl alcohol or hydrolyzed vinyl ester constituent, the percent by weight of which is indicated by the letter  $a$ , and the second member being the ethylene constituent, the per cent by weight of which is indicated by the letter  $b$ , the minimum tension to be applied is such that the increase in length in percent of the filaments is equal to  $190$  minus the product  $(18)b$ . The tension in grams per denier is equal to  $0.21$  minus the product  $(0.03)(b)$ . Thus, for polyvinyl alcohol itself, the tension should be such to produce an increase in length of at least  $190\%$  or at least  $0.21$  gram per denier. Less tension with correspondingly less orientation can be applied in the case of the hydrolyzed ethylene/vinyl ester interpolymers, but in any instance the minimum tension is such that the increase in length is at least  $100\%$  or must exceed  $0.05$  gram per denier. The maximum tension used naturally must be less than the breaking strength of the fiber. Although tensions near the maximum may be employed, such tensions may result in more broken filaments in the yarn than are desired. It is preferable to operate at tensions or length increases of about  $75\%$  of the maximum during the wet drawing. After drying the filaments, the fibers may be further oriented by drawing at elevated temperatures to give filaments having high tensile strength. The amount of this hot drawing is inversely proportional to the amount of wet drawing done during the spinning operation.

The fibers obtained by the process of this invention are particularly useful for the preparation of fabrics, cordage, etc. Aftertreatments with formaldehyde or other materials can be applied to the fibers to further reduce their water sensitivity. In view of the electrical insulating properties of hydrolyzed ethylene/vinyl acetate interpolymers, the fibers of such interpolymers may also be used in electrical insulation, e. g., for tape winding or braiding of electrical conductors.

As many apparently widely different embodiments of this invention may be made without departing from the spirit and scope thereof, it is to be understood that I do not limit myself

to the specific embodiments thereof except as defined in the appended claims.

I claim:

1. In the process for manufacture of filaments, fibers and like structures from a synthetic linear hydroxylated polymer wherein an aqueous solution of from 5% to 30% by weight of said polymer is coagulated in an aqueous solution of an inorganic salt, the improvement which comprises drawing the wet spun filaments at least twice their initial length under a tension which orients the filaments to an extent such that they do not stick together after washing with water alone and drying, holding the drawn filaments under tension at least twice their original length and while the filaments are so held washing them to remove said salt with an aqueous wash which consists essentially of water and which causes swelling of the filaments in their undrawn and unoriented state, and then drying the filaments while so held, said hydroxylated polymer having at least one alcoholic hydroxyl group per 2.5 carbon and not more than one hydroxyl per two carbons of the polymeric chain.
2. The process set forth in claim 1 in which said hydroxylated polymer consists predominantly of hydrolyzed polyvinyl ester.
3. The process set forth in claim 1 in which said hydroxylated polymer consists predominantly of hydrolyzed polyvinyl acetate.
4. The process set forth in claim 1 in which said hydroxylated polymer is a hydrolyzed ethylene/vinyl acetate interpolymer containing from 0.12% to 10% ethylene in the hydrolyzate.
5. The process set forth in claim 1 in which said salt is monosodium dihydrogen phosphate.

EDWARD TERRY CLINE.

#### REFERENCES CITED

- 40 The following references are of record in the file of this patent:

#### UNITED STATES PATENTS

| Number       | Name     | Date          |
|--------------|----------|---------------|
| 45 2,146,295 | Herrmann | Feb. 7, 1939  |
| 2,190,265    | Hubert   | Feb. 13, 1940 |
| 2,236,061    | Izard    | Mar. 25, 1941 |
| 2,322,976    | Schmitz  | June 29, 1943 |
| 50 2,388,325 | Houtz    | Nov. 6, 1945  |

#### FOREIGN PATENTS

| Number  | Country       | Date          |
|---------|---------------|---------------|
| 482,216 | Great Britain | Mar. 25, 1938 |